

United States Patent [19]  
Benedyk

[11] 4,356,220  
[45] \* Oct. 26, 1982

[54] ARTIFICIAL TURF-LIKE PRODUCT OF THERMOPLASTIC POLYMERS

[75] Inventor: Joseph C. Benedyk, Highland Park, Ill.

[73] Assignee: Brunswick Corporation, Skokie, Ill.

[\*] Notice: The portion of the term of this patent subsequent to Oct. 28, 1997, has been disclaimed.

[21] Appl. No.: 168,363

[22] Filed: Jul. 10, 1980

Related U.S. Application Data

[63] Continuation of Ser. No. 33,483, Apr. 26, 1979, abandoned.

[51] Int. Cl.<sup>3</sup> ..... A41G 1/00

[52] U.S. Cl. ..... 428/17; 428/92;  
428/97

[58] Field of Search ..... 428/17, 92, 97

[56]

References Cited

U.S. PATENT DOCUMENTS

|           |         |                 |        |
|-----------|---------|-----------------|--------|
| 3,332,828 | 7/1967  | Faria .....     | 428/17 |
| 3,513,062 | 5/1970  | Vinicki .....   | 428/17 |
| 3,551,263 | 12/1970 | Carter .....    | 428/17 |
| 3,837,980 | 9/1974  | Nishimura ..... | 428/17 |
| 3,940,522 | 2/1976  | Wessells .....  | 428/92 |
| 3,987,228 | 10/1976 | Hemming .....   | 428/92 |
| 4,061,804 | 12/1977 | McCulloch ..... | 428/17 |
| 4,104,428 | 8/1978  | Liu .....       | 428/97 |
| 4,230,752 | 10/1980 | Benedyk .....   | 428/17 |

Primary Examiner—Marion McCamish

Attorney, Agent, or Firm—John G. Heimovics

[57]

ABSTRACT

An artificial grass product with pile fibers having a modulus of elasticity of from 25,000 p.s.i. to 100,000 p.s.i. and a moment of inertia of from  $1.06 \times 10^{-10}$  in.<sup>4</sup> to  $8.33 \times 10^{-9}$  in.<sup>4</sup>. For fibers of rectangular cross-section the fiber dimensions range from 0.004 in. to 0.010 in. in thickness and 0.020 in. to 0.100 in. in width.

18 Claims, 3 Drawing Figures





FIG. 1



FIG. 2



FIG. 3

## ARTIFICIAL TURF-LIKE PRODUCT OF THERMOPLASTIC POLYMERS

This is a continuation, of application Ser. No. 5 033,483, filed on Apr. 26, 1979 now abandoned.

### CROSS-REFERENCE TO RELATED APPLICATIONS

This application is related to copending application 10 Ser. No. 17,465 of Joseph C. Benedyk, now abandoned, which is incorporated herein by reference.

This invention relates to an artificial grass product which simulates natural grass to a higher degree than commercially available artificial grasses. 15

### BACKGROUND OF THE INVENTION

All of the commercially available fibers for the manufacture of artificial grass are made of either fibrillated or slit polypropylene, polyamides, polyesters, etc. Those 20 fibers are typically made from a film of 0.0015 to 0.002 inches (in.) thickness. It is known that the artificial grass pile fabric made from these materials has several disadvantages, including: a stiffness parameter inconsistent with the "feel" of natural grass, poor matting resistance, 25 poor abrasion resistance, poor flammability qualities and poor ultraviolet resistance.

### OBJECTS OF THE INVENTION

An object of the present invention is to provide artificial grass fiber, yarn and pile products made therefrom that closely simulate the "feel" and look of natural grass and do not suffer from the deficiencies of commercially 30 available grass yarns and artificial grasses.

Another object of this invention is to provide a single 35 fiber pile product made of fibers comprising particular polymers and having a low elastic modulus and an area moment of inertia within a defined range.

A further object of this invention is to provide an 40 artificial grass product having fibers with a modulus of elasticity and an area moment of inertia closely approximating those properties of blades of Kentucky Blue Grass.

Still another object of the present invention is to provide an artificial grass product having superior ultraviolet 45 stability and weathering resistance in the absence or presence of an ultraviolet stabilizer or antioxidant.

A further object of the present invention is to provide an 50 artificial grass containing additives, such as ultraviolet stabilizers or antioxidants, to improve ultraviolet stability and weathering resistance.

Yet another object of the present invention is to provide an artificial grass product made from particular polymers in order to achieve the above-described objects and advantages. 55

### SUMMARY OF THE INVENTION

The artificial grass product of the present invention is made of yarn comprised of fibers or a single fiber having an elastic modulus of from 25,000 pounds/inch<sup>2</sup> (p.s.i.) to 100,000 p.s.i. and a moment of inertia about the x- or y-axis of from  $1.06 \times 10^{-10}$  inch<sup>4</sup> (in.<sup>4</sup>) to  $8.33 \times 10^{-9}$  in.<sup>4</sup>. The yarn of the invention is manufactured by extrusion/spinning through spinnerettes or by slitting or a polymer film. For specific details of this process reference is made to copending Benedyk application Ser. No. 17,465, now U.S. Pat. No. 4,181,762 previously referred to. 60

The elastic modulus and moment of inertia properties of the fibers of this invention allow use of yarn having substantially thicker fibers than are currently used in the art. Furthermore, the yarn may contain a mixture of fibers having varying cross-sectional shapes, elastic moduli and/or area moments of inertia. The yarn may be either twisted or braided from any number of the fibers described above.

Alternatively, the pile product of the invention may be made from single fibers having the properties described above.

The fibers of the artificial grass products of the invention closely simulate blades of Kentucky Blue Grass with respect to breaking load, ultimate tensile strength and elastic modulus. A turf product made with these fibers provides a surface more closely resembling natural grass than any conventional artificial grass product. 15

The invention may be better understood by reference to the appended drawings in which:

FIG. 1 is a cross-sectional view of a synthetic turf made by conventional methods using a braided yarn comprising fibers of the present invention.

FIG. 2 is a perspective view of a synthetic turf made by conventional methods using single fibers of the invention. 20

FIG. 3 is a cross-sectional view of the turf of FIG. 2 taken through section line 3'-3' of FIG. 2. 25

### THE FIBERS

The fibers of the invention may be of rectangular, triangular or circular cross-section or combinations thereof. The fibers have an elastic modulus of from 25,000 p.s.i. to 100,000 p.s.i. and an area moment of inertia ( $bh^3/12$ , where b is width and h is thickness of a rectangular cross-section taken perpendicular to the longitudinal axis of the fiber) of from  $1.06 \times 10^{-10}$  to  $8.33 \times 10^{-9}$  in.<sup>4</sup>. For a rectangular cross-section, the fiber dimensions should range from 0.004 in. to 0.010 in. in thickness and 0.020 in. to 0.100 in. in width. These fibers may be extruded from commercially available polymers, including: ethylene-vinyl acetate copolymers, plasticized polyvinyl chloride, low density polyethylene, ethylene-ethyl acrylate copolymer, ethylenebutylene copolymer, polybutylene and various copolymers thereof, certain ethylene-propylene copolymers, chlorinated polypropylene, chlorinated polybutylene and various compatible mixtures of these thermoplastics. The prior art has consistently viewed these polymers as unsuitable for use in fibers precisely because of their low elastic modulus and also because of their uniformly low tensile strength.

U.S. Pat. No. 3,573,147, which is incorporated herein by reference, discusses a method of making suitable ribbon-shaped fibers which may be used to produce the fibers of the invention. 55

The ribbon-like fibers can be made by extrusion from a rectangular, slotted orifice dimensioned to produce fibers having a thickness of between 0.004 in. and 0.010 in. and a width of between 0.020 in. and 0.100 in. since fibers having these cross-sectional dimensions possess good flexing and bending characteristics. However, as noted above, the cross-sections need not be rectangular-shaped. Where the fibers have a generally circular cross-section, the diameter may be from about 0.003 in. to 0.006 in. 60

The ribbon-like fibers can also be made by slitting of plastic film or sheet having a thickness of between 0.004

in. and 0.010 in. to a fiber width of between 0.020 in. and 0.100 in.

### CROSS-LINKING

It is also desirable to cross-link the fibers by use of ionizing radiation, such as gamma rays emitted by radioactive elements and isotopes, x-rays, rays of subatomic charged particles including electrons, protons, deuterons, and rays of neutrons.

The dosage of radiation should be sufficient to cross-link the molecules to the extent that they have a gel content greater than 30% but less than 90%. The preferred gel content is 45-55%. Gel content of the ethylene-vinyl acetate fiber, for example, is determined according to the following procedure:

Fibers are wound around a metal wire screen and subjected to solvent elution in hot xylene near the boiling point for 24 hours. Gel content is then calculated using the formula:

$$\% \text{ gel} = \frac{W_f - W_o}{W_o} \times 100$$

Where  $W_o$  is the initial weight of the sample and  $W_f$  is the final weight after elution.

To enhance cross-linking there may be distributed throughout the polymeric material fine particles of silicon dioxide, titanium dioxide or some other inorganic filler which enhances radiation cross-linking. The particle size of these oxides ranges between 100 angstroms and 1 micron and the amount used is below 1 volume percent. This small amount of inorganic filler improves the efficiency of the irradiation step. For example, a polymeric material irradiated at a dosage of 10 megarads (MR) will have a gel content of 25-28%. When this same polymer includes 0.2 volume percent silicon dioxide and is irradiated at the same dosage, the gel content is 40-45%. This increase in gel content represents a substantial increase in the melting point of the polymeric material. The addition of polyfunctional monomers also improves cross-linking. For example, triallyl cyanurate or triallyl acylate, alone or in combination with the oxides, are additives which enhance the cross-linking yield for a given radiation dosage.

The thermoplastic materials of the invention may be cross-linked before, during or after the fibers are formed, or during or after the pile fabric is made. Miltz and Narkis (J. Appl. Polymer Sci. 20: 1627-1633 (1976)) have described the synergistic effect which occurs when cross-linking, such as described above, and ultraviolet stabilization are combined in raising the ultraviolet resistance of low density polyethylene.

### THE YARN

The yarn can be made by extrusion, by direct attenuation in the melt to final cross-sectional shape; by combined melt attenuation and solid phase drawing, or by slitting of solid film. The yarn may consist of a combination of fibers having various cross-sectional shapes or dimensions.

Braiding or twisting of the fibers may be accomplished on any conventional braiding or twisting machine as, for example, one designed which accommodates from 4 to 8 carriers. The desired flexibility of the braided yarn for conventional tufting makes it preferable that no central fiber be included in the braid when it is subjected to tufting. Any conventional tufting technique may be used with the braided or twisted filaments. When tension is applied to the yarn by the machine during tufting, all of the ends pull together into a

5  
10  
15

4  
tight yarn which easily passes through the machine elements.

### THE PILE TURF

A detailed description of the production of artificial grass made from ribbon-like fibers can be found in U.S. Pat. No. 3,551,263, which is incorporated herein by reference. Basically, the invention described therein provides a cut pile-type synthetic turf having fibers of substantially rectangular cross-section.

Also discussed therein is a method of preparing a yarn consisting of the above-described fibers suitable for conventional cut pile tufting in the production of synthetic turf. Four to eight of the fibers are braided or twisted into a yarn which is secured by conventional cut pile tufting, weaving, knitting, or otherwise to form a structure consisting of a backing having a cut pile face extending from one surface thereof. Where tufting, knitting or weaving is employed, a suitable latex formulation is applied to the other surface of the backing to render the complete structure dimensionally stable. A polymeric elastomer may then be applied to the latex backing to provide a more stable and improved structure.

20  
25  
30  
35  
40  
45  
50  
55  
60

FIG. 1 is a cross-sectional view of a synthetic turf produced by the conventional methods discussed in U.S. Pat. No. 3,551,263 using a braided yarn. Fibers 1 emerge from the fiber backing 2, the pile being anchored securely therein by a bonding agent 3. A polyvinyl chloride foam 4 has been applied to the backing to improve the physical properties of the turf.

In another embodiment, a single fiber pile is used in making the synthetic turf (see FIGS. 2 and 3) according to the process described in U.S. Pat. No. 3,332,828. A portion of the woven turf 5 is shown in which single fibers 6 extend upwardly from a woven synthetic fiber backing 7. The fibers 6 are anchored securely in the backing 7 by a bonding agent 8. A polyvinyl chloride foam 9 is applied on the backing 7 to improve the physical properties of the turf 5.

### FIBER PROPERTIES

The mechanical properties of the low modulus, large diameter fibers of the invention were compared to the mechanical properties of blades of Kentucky Blue Grass as follows:

#### Tensile Test

50  
55  
60  
65

A table model Instron testing machine was used with Instron's "C" load cell at one pound (lb.) full scale deflection for the Kentucky Blue Grass with a cross-head speed of 0.2 inch/minute (in./min.), chart speed of 1 in./min. and a gauge length of 2 in. The fibers of the invention were tested in the same way with the exception of having the load cell at 2 lb. full scale deflection and a cross-head speed of 2 in./min., chart speed of 1 in./min., and a 2 in. gauge length.

#### Bending Modulus Test

The same Instron machine was used as previously described with the exception of a different gripping arrangement. The load cell used was an "A" cell at 10 grams full-scale deflection, 0.2 in./min. cross-head speed, 10 in./min. chart speed, and 1 in. gauge length.

65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
340  
341  
342  
343  
344  
345  
346  
347  
348  
349  
350  
351  
352  
353  
354  
355  
356  
357  
358  
359  
360  
361  
362  
363  
364  
365  
366  
367  
368  
369  
370  
371  
372  
373  
374  
375  
376  
377  
378  
379  
380  
381  
382  
383  
384  
385  
386  
387  
388  
389  
390  
391  
392  
393  
394  
395  
396  
397  
398  
399  
400  
401  
402  
403  
404  
405  
406  
407  
408  
409  
410  
411  
412  
413  
414  
415  
416  
417  
418  
419  
420  
421  
422  
423  
424  
425  
426  
427  
428  
429  
430  
431  
432  
433  
434  
435  
436  
437  
438  
439  
440  
441  
442  
443  
444  
445  
446  
447  
448  
449  
450  
451  
452  
453  
454  
455  
456  
457  
458  
459  
460  
461  
462  
463  
464  
465  
466  
467  
468  
469  
470  
471  
472  
473  
474  
475  
476  
477  
478  
479  
480  
481  
482  
483  
484  
485  
486  
487  
488  
489  
490  
491  
492  
493  
494  
495  
496  
497  
498  
499  
500  
501  
502  
503  
504  
505  
506  
507  
508  
509  
510  
511  
512  
513  
514  
515  
516  
517  
518  
519  
520  
521  
522  
523  
524  
525  
526  
527  
528  
529  
530  
531  
532  
533  
534  
535  
536  
537  
538  
539  
540  
541  
542  
543  
544  
545  
546  
547  
548  
549  
550  
551  
552  
553  
554  
555  
556  
557  
558  
559  
5510  
5511  
5512  
5513  
5514  
5515  
5516  
5517  
5518  
5519  
5520  
5521  
5522  
5523  
5524  
5525  
5526  
5527  
5528  
5529  
5530  
5531  
5532  
5533  
5534  
5535  
5536  
5537  
5538  
5539  
5540  
5541  
5542  
5543  
5544  
5545  
5546  
5547  
5548  
5549  
5550  
5551  
5552  
5553  
5554  
5555  
5556  
5557  
5558  
5559  
5560  
5561  
5562  
5563  
5564  
5565  
5566  
5567  
5568  
5569  
55610  
55611  
55612  
55613  
55614  
55615  
55616  
55617  
55618  
55619  
55620  
55621  
55622  
55623  
55624  
55625  
55626  
55627  
55628  
55629  
55630  
55631  
55632  
55633  
55634  
55635  
55636  
55637  
55638  
55639  
55640  
55641  
55642  
55643  
55644  
55645  
55646  
55647  
55648  
55649  
55650  
55651  
55652  
55653  
55654  
55655  
55656  
55657  
55658  
55659  
55660  
55661  
55662  
55663  
55664  
55665  
55666  
55667  
55668  
55669  
55670  
55671  
55672  
55673  
55674  
55675  
55676  
55677  
55678  
55679  
55680  
55681  
55682  
55683  
55684  
55685  
55686  
55687  
55688  
55689  
55690  
55691  
55692  
55693  
55694  
55695  
55696  
55697  
55698  
55699  
556100  
556101  
556102  
556103  
556104  
556105  
556106  
556107  
556108  
556109  
556110  
556111  
556112  
556113  
556114  
556115  
556116  
556117  
556118  
556119  
556120  
556121  
556122  
556123  
556124  
556125  
556126  
556127  
556128  
556129  
556130  
556131  
556132  
556133  
556134  
556135  
556136  
556137  
556138  
556139  
556140  
556141  
556142  
556143  
556144  
556145  
556146  
556147  
556148  
556149  
556150  
556151  
556152  
556153  
556154  
556155  
556156  
556157  
556158  
556159  
556160  
556161  
556162  
556163  
556164  
556165  
556166  
556167  
556168  
556169  
556170  
556171  
556172  
556173  
556174  
556175  
556176  
556177  
556178  
556179  
556180  
556181  
556182  
556183  
556184  
556185  
556186  
556187  
556188  
556189  
556190  
556191  
556192  
556193  
556194  
556195  
556196  
556197  
556198  
556199  
556200  
556201  
556202  
556203  
556204  
556205  
556206  
556207  
556208  
556209  
556210  
556211  
556212  
556213  
556214  
556215  
556216  
556217  
556218  
556219  
556220  
556221  
556222  
556223  
556224  
556225  
556226  
556227  
556228  
556229  
556230  
556231  
556232  
556233  
556234  
556235  
556236  
556237  
556238  
556239  
556240  
556241  
556242  
556243  
556244  
556245  
556246  
556247  
556248  
556249  
556250  
556251  
556252  
556253  
556254  
556255  
556256  
556257  
556258  
556259  
556260  
556261  
556262  
556263  
556264  
556265  
556266  
556267  
556268  
556269  
556270  
556271  
556272  
556273  
556274  
556275  
556276  
556277  
556278  
556279  
556280  
556281  
556282  
556283  
556284  
556285  
556286  
556287  
556288  
556289  
556290  
556291  
556292  
556293  
556294  
556295  
556296  
556297  
556298  
556299  
556300  
556301  
556302  
556303  
556304  
556305  
556306  
556307  
556308  
556309  
556310  
556311  
556312  
556313  
556314  
556315  
556316  
556317  
556318  
556319  
556320  
556321  
556322  
556323  
556324  
556325  
556326  
556327  
556328  
556329  
556330  
556331  
556332  
556333  
556334  
556335  
556336  
556337  
556338  
556339  
556340  
556341  
556342  
556343  
556344  
556345  
556346  
556347  
556348  
556349  
556350  
556351  
556352  
556353  
556354  
556355  
556356  
556357  
556358  
556359  
556360  
556361  
556362  
556363  
556364  
556365  
556366  
556367  
556368  
556369  
556370  
556371  
556372  
556373  
556374  
556375  
556376  
556377  
556378  
556379  
556380  
556381  
556382  
556383  
556384  
556385  
556386  
556387  
556388  
556389  
556390  
556391  
556392  
556393  
556394  
556395  
556396  
556397  
556398  
556399  
556400  
556401  
556402  
556403  
556404  
556405  
556406  
556407  
556408  
556409  
556410  
556411  
556412  
556413  
556414  
556415  
556416  
556417  
556418  
556419  
556420  
556421  
556422  
556423  
556424  
556425  
556426  
556427  
556428  
556429  
556430  
556431  
556432  
556433  
556434  
556435  
556436  
556437  
556438  
556439  
556440  
556441  
556442  
556443  
556444  
556445  
556446  
556447  
556448  
556449  
556450  
556451  
556452  
556453  
556454  
556455  
556456  
556457  
556458  
556459  
556460  
556461  
556462  
556463  
556464  
556465  
556466  
556467  
556468  
556469  
556470  
556471  
556472  
556473  
556474  
556475  
556476  
556477  
556478  
556479  
556480  
556481  
556482  
556483  
556484  
556485  
556486  
556487  
556488  
556489  
556490  
556491  
556492  
556493  
556494  
556495  
556496  
556497  
556498  
556499  
556500  
556501  
556502  
556503  
556504  
556505  
556506  
556507  
556508  
556509  
556510  
556511  
556512  
556513  
556514  
556515  
556516  
556517  
556518  
556519  
556520  
556521  
556522  
556523  
556524  
556525  
556526  
556527  
556528  
556529  
556530  
556531  
556532  
556533  
556534  
556535  
556536  
556537  
556538  
556539  
556540  
556541  
556542  
556543  
556544  
556545  
556546  
556547  
556548  
556549  
556550  
556551  
556552  
556553  
556554  
556555  
556556  
556557  
556558  
556559  
556560  
556561  
556562  
556563  
556564  
556565  
556566  
556567  
556568  
556569  
556570  
556571  
556572  
556573  
556574  
556575  
556576  
556577  
556578  
556579  
556580  
556581  
556582  
556583  
556584  
556585  
556586  
556587  
556588  
556589  
556590  
556591  
556592  
556593  
556594  
556595  
556596  
556597  
556598  
556599  
556600  
556601  
556602  
556603  
556604  
556605  
556606  
556607  
556608  
556609  
556610  
556611  
556612  
556613  
556614  
556615  
556616  
556617  
556618  
556619  
556620  
556621  
556622  
556623  
556624  
556625  
556626  
556627  
556628  
556629  
556630  
556631  
556632  
556633  
556634  
556635  
556636  
556637  
556638  
556639  
556640  
556641  
556642  
556643  
556644  
556645  
556646  
556647  
556648  
556649  
556650  
556651  
556652  
556653  
556654  
556655  
556656  
556657  
556658  
556659  
556660  
556661  
556662  
556663  
556664  
556665  
556666  
556667  
556668  
556669  
556670  
556671  
556672  
556673  
556674  
556675  
556676  
556677  
556678  
556679  
556680  
556681  
556682  
556683  
556684  
556685  
556686  
556687  
556688  
556689  
556690  
556691  
556692  
556693  
556694  
556695  
556696  
556697  
556698  
556699  
556700  
556701  
556702  
556703  
556704  
556705  
556706  
556707  
556708  
556709  
556710  
556711  
556712  
556713  
556714  
556715  
556716  
556717  
556718  
556719  
556720  
556721  
556722  
556723  
556724  
556725  
556726  
556727  
556728  
556729  
556730  
556731  
556732  
556733  
556734  
556735  
556736  
556737  
556738  
556739  
556740  
556741  
556742  
556743  
556744  
556745  
556746  
556747  
556748  
556749  
556750  
556751  
556752  
556753  
556754  
556755  
556756  
556757  
556758  
556759  
556760  
556761  
556762  
556763  
556764  
556765  
556766  
556767  
556768  
556769  
556770  
556771  
556772  
556773  
556774  
556775  
556776  
556777  
556778  
556779  
556780  
556781  
556782  
556783  
556784  
556785  
556786  
556787  
556788  
556789  
5567

fibers used in the prior art to make artificial turf. Table II presents the parameters relating to measurement of the bending modulus.

TABLE I

## SUMMARY OF TENSILE PROPERTIES

| Specimen                                  | Cross-Sectional Area (in. <sup>2</sup> ) | Breaking Load (lb.) | Ultimate Tensile Strength (10 <sup>3</sup> psi) | Elastic Modulus (10 <sup>3</sup> psi) | % Elongation in 2 in. |
|-------------------------------------------|------------------------------------------|---------------------|-------------------------------------------------|---------------------------------------|-----------------------|
| <u>Kentucky Grass</u>                     |                                          |                     |                                                 |                                       |                       |
| #1                                        | .00024                                   | .35                 | 1.4                                             | 41.7*                                 |                       |
| #2                                        | .00028                                   | .57                 | 2.0                                             | 50.9                                  |                       |
| #3                                        | .00012                                   | .55                 | 4.5                                             | 61.6                                  |                       |
| #4                                        | .00028                                   | .90                 | 3.2                                             | 45.9                                  |                       |
| #5                                        | .00012                                   | .17                 | 1.4                                             | 94.4                                  |                       |
| #6                                        | .00024                                   | .17                 | 0.70                                            | 35.4                                  |                       |
| #7                                        | .00028                                   | .60                 | 2.1                                             | 61.2                                  |                       |
| #8                                        | .00028                                   | .63                 | 2.2                                             | 56.2                                  |                       |
| #9                                        | .00028                                   | .27                 | 0.96                                            | 27.5                                  |                       |
| #10                                       | .00024                                   | .37                 | 1.5                                             | 51.4                                  |                       |
| <u>Drawn Fiber</u>                        |                                          |                     |                                                 |                                       |                       |
| Run #2                                    |                                          |                     |                                                 |                                       |                       |
| #1                                        | .000328                                  | 1.04                | 3.1                                             | 79                                    | 176                   |
| #2                                        | .000328                                  | 1.00                | 3.0                                             | 61                                    | 183                   |
| #3                                        | .000328                                  | 1.02                | 3.1                                             | 75.8                                  | 148                   |
| <u>Extruded Fiber</u>                     |                                          |                     |                                                 |                                       |                       |
| Run #1                                    |                                          |                     |                                                 |                                       |                       |
| #1                                        | .000664                                  | 1.34                | 2.0                                             | 53.2                                  | 218                   |
| #2                                        | .000547                                  | 1.09                | 1.9                                             | 65                                    | 197                   |
| #3                                        | .000664                                  | 1.52                | 2.2                                             | 59                                    | 303                   |
| <u>Extruded Fiber</u>                     |                                          |                     |                                                 |                                       |                       |
| Run #2                                    |                                          |                     |                                                 |                                       |                       |
| #1                                        | .000469                                  | 1.05                | 2.2                                             | 66.3                                  | 215                   |
| #2                                        | .000469                                  | 1.07                | 2.2                                             | 68.2                                  | 180                   |
| #3                                        | .000500                                  | 1.10                | 2.2                                             | 64                                    | 228                   |
| <u>Polypropylene Fiber (Bundled-Yarn)</u> |                                          |                     |                                                 |                                       |                       |
| #1                                        | .001265                                  | 37.5                | 34                                              | 225                                   | 93                    |
| #2                                        | .001265                                  | 40                  | 36                                              | 263                                   | 77                    |
| #3                                        | .001265                                  | 46                  | 42                                              | 197                                   | 110                   |

\*Low values for data of ELASTIC MODULUS VS. values for BENDING MODULUS of the natural grass may be attributed to samples breaking near the grip.

TABLE II

## BENDING MODULUS

| Sample                                                              | h (in.) | b (in.) | $\delta$ (in.) | P (10 <sup>-5</sup> lb.) | I (in.) | I (10 <sup>-9</sup> in. <sup>4</sup> ) | E (10 <sup>3</sup> psi) | K (10 <sup>-5</sup> lb.-in. <sup>2</sup> ) |
|---------------------------------------------------------------------|---------|---------|----------------|--------------------------|---------|----------------------------------------|-------------------------|--------------------------------------------|
| <u>Drawn Fibers</u>                                                 |         |         |                |                          |         |                                        |                         |                                            |
| Run #3                                                              |         |         |                |                          |         |                                        |                         |                                            |
| #1                                                                  | .0075   | .0625   | .06            | 44.05                    | .5      | 2.196                                  | 141                     | 30.97                                      |
| #2                                                                  | .0075   | .0625   | .08            | 27.50                    | .5      | 2.196                                  | 65.2                    | 14.32                                      |
| #3                                                                  | .0075   | .0625   | .10            | 33.00                    | .5      | 2.196                                  | 65.2                    | 13.67                                      |
| #4                                                                  | .0080   | .0625   | .08            | 22.02                    | .5      | 2.666                                  | 43                      | 11.46                                      |
| #5                                                                  | .0080   | .0625   | .08            | 22.02                    | .5      | 2.666                                  | 43                      | 11.46                                      |
| <u>Kentucky Blue Grass</u>                                          |         |         |                |                          |         |                                        |                         |                                            |
| #1                                                                  | .0060   | .0859   | .08            | 33.03                    | .5      | 1.546                                  | 110                     | 17.20                                      |
| #2                                                                  | .0060   | .0937   | .07            | 55.06                    | .5      | 1.686                                  | 194                     | 32.77                                      |
| #3                                                                  | .0060   | .0937   | .07            | 44.05                    | .5      | 1.686                                  | 155                     | 26.22                                      |
| #4                                                                  | .0060   | .10937  | .06            | 88.10                    | .5      | 1.968                                  | 305                     | 60.17                                      |
| #5                                                                  | .0060   | .10937  | .07            | 66.07                    | .5      | 1.968                                  | 199                     | 39.33                                      |
| <u>Polypropylene (Bundled Synthetic Grass Yarn - Thiokol Corp.)</u> |         |         |                |                          |         |                                        |                         |                                            |
| #1                                                                  | .013    | .0937   | .0385          | 616.7                    | .5      | 17.154                                 | 389                     | 667.42                                     |
| #2                                                                  | .014    | .0937   | .0230          | 638.7                    | .5      | 21.426                                 | 540                     | 1,157.00                                   |
| <u>Drawn Fibers</u>                                                 |         |         |                |                          |         |                                        |                         |                                            |
| Run #2                                                              |         |         |                |                          |         |                                        |                         |                                            |
| #1                                                                  | .007    | .0625   | .09            | 22.02                    | .5      | 1.786                                  | 57                      | 10.198                                     |
| #2                                                                  | .007    | .0625   | .09            | 22.02                    | .5      | 1.786                                  | 57                      | 10.198                                     |
| <u>Extruded Fibers</u>                                              |         |         |                |                          |         |                                        |                         |                                            |
| Run #2                                                              |         |         |                |                          |         |                                        |                         |                                            |
| #1                                                                  | .008    | .0625   | .09            | 33.03                    | .5      | 2.666                                  | 57                      | 15.292                                     |
| #2                                                                  | .008    | .0625   | .07            | 33.03                    | .5      | 2.666                                  | 73                      | 19.660                                     |

b = width of sample

h = thickness of sample

P = load placed on sample

 $\delta$  = amount of deflection

I = lever arm

I = the moment of inertia of a rectangular specimen ( $bh^3/12$ ) $E = PI^3/3I$ K =  $E \times I$  (stiffness parameter)

## EXAMPLE I

A synthetic poly(ethylene-vinyl acetate) turf was produced by tufting a 6 ply twisted yarn comprised of fibers of rectangular cross-section with dimensions 0.004 in.  $\times$  0.080 in. The fibers have an elastic modulus of about 80,000 p.s.i. and an area moment of inertia of about  $4.0 \times 10^{-9}$  in.<sup>4</sup>. The fibers were inserted into a backing of a  $\frac{1}{8}$  in. thick sheet of polyurethane foam which was reinforced by a nylon scrim. The tufts were cut to form a turf with a pile height of  $\frac{3}{8}$  in. and the back of the fabric was latexed to firmly anchor the nylon and prevent shedding.

## EXAMPLE II

The flat fibers of Example I were tufted into standard Chemback tufting medium and sheared to  $\frac{1}{4}$  in. pile height with 18 ounces of fiber per square yard of fabric. A latex adhesive was applied to the underside of a portion of the fabric and a non-woven rayon-polyolefin scrim was applied to the adhesive to form a secondary backing.

What is claimed:

1. An artificial grass product, comprising: a pile fabric with yarn comprised of a plurality of fibers made of a polymeric material selected from the group consisting of copolymers of ethylene-vinyl acetate, ethylene-ethyl acrylate, ethylene-butylene, ethylene-propylene; polyvinyl chloride; chlorinated polyolefins; low density polyethylene; and mixtures thereof and having an elastic modulus of from 25,000 p.s.i. to 100,000 p.s.i. and a moment of inertia of from  $1.06 \times 10^{-10}$  in.<sup>4</sup> to  $8.33 \times 10^{-9}$  in.<sup>4</sup>, the fibers extending from and substantially perpendicular to a backing to which the fibers are secured, wherein the yarn is twisted at the point of emergence from the backing.
2. The artificial grass product of claim 1, wherein the

fibers have a rectangular cross-section of from 0.004 in. to 0.010 in. in thickness and from 0.020 in. to 0.100 in. in width.

3. The artificial grass product of claim 2, wherein the polymeric material has dispersed therein an additive selected from the group consisting of colorants, fillers, flame retardants, ultraviolet stabilizers, antioxidants, antistatic agents and antisoiling agents.

4. The artificial grass product of claim 2, wherein the polymeric material contains an antioxidant.

5. The artificial grass product of claim 2, wherein the polymeric material contains an ultraviolet stabilizer.

6. The artificial grass product of claim 1, wherein the fibers have a generally circular cross-section of from 0.003 to 0.006 in. in diameter.

7. The artificial grass product of claim 1, wherein the fibers are tufted into the backing.

8. The artificial grass product of claim 1, wherein the fibers are woven into a warp and fill backing.

9. The artificial grass product of claim 1, wherein the fibers are knitted with the fibers of the backing.

10. An artificial grass product, comprising: a pile fabric with yarn comprised of a single fiber made of a polymeric material selected from the group consisting of copolymers of ethylene-vinyl acetate, ethylene-ethyl acrylate, ethylene-butylene, ethylene-propylene; polyvinyl chloride; chlorinated polyolefins; low density

polyethylene; and mixtures thereof and having an elastic modulus of from 25,000 p.s.i. to 100,000 p.s.i. and a moment of inertia of from  $1.06 \times 10^{-10}$  in.<sup>4</sup> to  $8.33 \times 10^{-9}$  in.<sup>4</sup>, the yarn tufted into a backing to form successive rows of loops of the fiber which are cut to provide a cut-pile face.

11. The artificial grass product of claim 10, wherein the fibers have a rectangular cross-section of from 0.004 in. to 0.010 in. in thickness and from 0.020 in. to 0.100 in. in width.

12. The artificial product of claim 11, wherein the polymeric material has dispersed therein an additive selected from the group consisting of colorants, fillers, flame retardants, ultraviolet stabilizers, antioxidants, antistatic agents and antisoiling agents.

13. The artificial grass product of claim 11, wherein the polymeric material contains an antioxidant.

14. The artificial grass product of claim 11, wherein the polymeric material contains an ultraviolet stabilizer.

15. The artificial grass product of claim 10, wherein the fibers have a generally circular cross-section of from 0.003 to 0.006 in. in diameter.

16. The artificial grass product of claim 10, wherein the fibers are tufted into the backing.

17. The artificial grass product of claim 10, wherein the fibers are woven into a warp and fill backing.

18. The artificial grass product of claim 10, wherein the fibers are knitted with the fibers of the backing.

\* \* \* \* \*

30

35

40

45

50

55

60

65